

# UNITED STATES PATENT OFFICE.

GEORGE O. SEWARD AND FRANZ VON KÜGELGEN, OF HOLCOMBS ROCK, VIRGINIA, ASSIGNORS  
TO VIRGINIA LABORATORY COMPANY, OF NEW YORK, N. Y., A CORPORATION OF NEW  
YORK.

## ELECTROLYTIC PRODUCTION OF MAGNESIUM.

No. 931,092.

Specification of Letters Patent.

Patented Aug. 17, 1909.

Application filed March 28, 1906. Serial No. 308,454.

*To all whom it may concern:*

Be it known that we, GEORGE O. SEWARD,  
a citizen of the United States, and FRANZ  
VON KÜGELGEN, a subject of the German  
Emperor, both residing at Holcombs Rock,  
in the county of Bedford and State of Vir-  
ginia, have jointly invented certain new and  
useful Improvements in the Electrolytic Pro-  
duction of Magnesium, of which the follow-  
ing is a specification.

This invention relates to the production  
of magnesium by electrolysis of its fused  
salts. Such electrolysis affords serious dif-  
ficulty, because the difference in the specific  
gravity of the liberated metal differs so  
slightly from that of its fused salt, that the  
metal does not readily separate. It is prac-  
tically necessary for good results to use an  
electrolyte whose specific gravity is so dif-  
ferent from that of magnesium, that the lat-  
ter will either sink readily to the bottom or  
rise freely to the top of the bath, where it  
can be collected. For a metal as light as  
magnesium it is extremely difficult to find  
electrolytes which have so low a specific  
gravity that the separated metal will readily  
sink to the bottom, and in such cases it is  
preferable to add to the electrolyte a com-  
ponent which will make it materially  
heavier than the metal, so that the latter  
will rise to the top of the bath. Such added  
component should be a flux which is efficient  
when used in comparatively small quanti-  
ties, and should not be decomposed by the  
current.

The present invention is characterized by  
the use for this purpose of the salts of the  
alkali-earth metals, which are peculiarly  
suited to this use because (1) they have a  
high specific gravity, and (2) they are dif-  
ficult to decompose electrolytically.

As an example of the practical application  
of our invention, we will describe the pro-  
duction of magnesium by electrolysis of  
magnesium chlorid, using barium chlorid to  
increase the specific gravity of the elec-  
trolyte.

At present magnesium is produced elec-  
trolytically from an electrolyte of fused

magnesium chlorid, with potassium chlorid  
added as a flux, the separated magnesium  
being collected at the bottom of the vessel.  
It is only under certain conditions of tem-  
perature that such an electrolyte is lighter  
than the separated magnesium, and it is dif-  
ficult to so manage the process that these  
temperature conditions are maintained so  
that a good separation of the magnesium re-  
sults.

In producing magnesium according to the  
present invention, we replace the potassium  
chlorid partly by barium chlorid, so that we  
obtain an electrolyte which is so much  
heavier than the magnesium, that the latter  
rises readily to the top, where it may be  
collected. Although the proportion of ba-  
rium chlorid may be greatly varied, we have  
found an electrolyte of the following com-  
position to give suitable results:— $MgCl_2$  5  
parts,  $KCl$  5 parts,  $BaCl_2$ , 3.5 parts.

Instead of barium chlorid we may use the  
chlorid or other suitable salt of calcium or  
strontium.

We are aware that alkali-earth salts have  
been used before as fluxes, but not for the  
purpose of regulating the specific gravity of  
the electrolyte.

What we claim is:—

1. The electrolytic production of mag-  
nesium by electrolyzing fused magnesium  
chlorid to which is added enough of a denser  
alkali-earth chlorid to render the bath  
heavier than the separated magnesium.

2. The electrolytic production of mag-  
nesium by electrolyzing a fused bath of  
magnesium chlorid and barium chlorid.

3. The electrolytic production of mag-  
nesium by electrolyzing a fused bath of mag-  
nesium chlorid, potassium chlorid, and  
barium chlorid.

In witness whereof, we have hereunto  
signed our names in the presence of two sub-  
scribing witnesses.

GEORGE O. SEWARD.

FRANZ VON KÜGELGEN.

Witnesses:

J. H. WEBB,

F. V. BINDER.